

April 7, 1970

R. L. LEONARD ET AL

3,505,445

SOLVENT REMOVAL PROCESS FOR WET SPUN FIBERS

Filed Nov. 17, 1967



INVENTORS

RICHARD L. LEONARD  
THOMAS B. TRUSCOTT  
THOMAS M. VEAZEY

BY

*Thomas M. Veazy*  
ATTORNEY

1

3,505,445  
**SOLVENT REMOVAL PROCESS FOR WET SPUN FIBERS**

Richard L. Leonard, Raleigh, N.C., and Thomas B. Truscott and Thomas M. Veazey, Decatur, Ala., assignors to Monsanto Company, St. Louis, Mo., a corporation of Delaware

Filed Nov. 17, 1967, Ser. No. 683,966  
 Int. Cl. B29b 11/22

U.S. Cl. 264—233

10 Claims

**ABSTRACT OF THE DISCLOSURE**

Substantially solvent free acrylic fibers are produced by washing with water and simultaneously stretching the newly formed fibers, in all instances at a maximum temperature of less than about 86° C. and, in some instances, at lower maximum temperatures depending upon the minimum orientation stretch ratio employed.

**BACKGROUND OF THE INVENTION**

This invention relates to fibers, filaments, yarns and the like manufactured from acrylonitrile polymers and to an improved process of producing the same. More particularly this invention relates to improvements in the process of removing solvents used in the polymerization of acrylonitrile polymers and in the coagulating bath following the spinning step in the production of acrylonitrile fibers, to thereby obtain a finished fiber with a minimum of residual solvent therein.

Since acrylonitrile polymers do not melt, filaments of such polymers are formed by dissolving the polymers in a suitable solvent and then removing the solvent from a flowing stream of the solution to form filaments therefrom. Commercially filaments of acrylonitrile polymers are prepared either by the dry spinning process or by the wet spinning process as is well known.

Ordinarily, in the wet spinning operation, coagulation is accomplished by extruding the polymer solution into an aqueous bath sometimes containing a percentage of solvent or dissolved salt. As used herein an aqueous or water bath refers to a composition using water as one of its main components. When the solvent is extracted from the extruded stream of spinning solution in a coagulating bath during wet spinning, solidification of the polymer in filamentary form results. The coagulating bath most frequently employed in the art is an aqueous bath employing a solvent, such as N,N-dimethylacetamide, N,N-dimethylformamide or the like, preferably the same solvent which is used to dissolve the polymer.

Instead of an aqueous coagulating bath, the art also teaches the use of a bath composed essentially of materials of such dissimilar character as butyl alcohol, kerosene and the polyalkylene glycols. Generally these baths contain less than 1% water, and with a tolerance of up to 20% of the solvent in which the polymer is dissolved. These coagulation baths are referred to as "nonaqueous" baths.

Most solvents used in the preparation of acrylonitrile spinning dopes are toxic and may impart an objectionable odor to the fiber. Residual solvents in the fibers also affect physical properties and dyeing characteristics of the fibers. Moreover, it is economically advantageous to remove all solvents from fibers for recovery and reuse.

Experience has shown that the presence of residual solvents in spun fibers has been greater or lesser depending upon the type of solvent used and upon the type of coagulation employed. Where coagulation is accomplished by extruding the solution into an aqueous bath which contains a percentage of solvent or dissolved salt, the residual

2

solvent in the fibers can usually be reduced to very low levels by washing and stretching the coagulated fibers in water at a temperature near boiling. This temperature usually conforms closely with required stretch temperatures for desired stretch ratios of fibers extruded into aqueous solutions. Where nonaqueous coagulation baths are used, for reasons unknown, difficulties in the removal of residual solvent become more pronounced, although stretching without breakage is more easily accomplished. Residual solvent after use of nonaqueous coagulation bath systems, following which the fibers are washed and stretched in the usual manner, in boiling or near boiling water, is 1% or higher.

**SUMMARY OF THE INVENTION**

It is an object of this invention to provide a process for the removal of substantially all residual solvents from fibers which have been made by spinning a solution of an acrylonitrile polymer in a solvent into any coagulating bath.

Other objects will become apparent from the following description of the invention and claims.

It has been found that unexpectedly improved results in the elimination of residual solvents are obtained by washing fibers in a bath or cascade of water the maximum critical temperature of which varies in accordance with the amount of stretch applied to the fiber (stretch ratio of the fiber) while in the wash.

These maximum critical temperatures are believed to be determined by the second order transition temperature, or glass temperature ( $T_g$ ) of the acrylonitrile copolymer. That is to say, the temperatures reflected in the following examples are believed to be just below the second order transition temperature of the acrylonitrile copolymer in each instance. Measured  $T_g$  values vary with the means used to determine  $T_g$ , and with the state of molecular order of the fibers. It is probable that fiber  $T_g$  depends upon fiber orientation and therefore upon degree of stretch or drawing. It is also probable that the presence of the solvent in the fibers at transition stages of molecular orientation lowers the  $T_g$ , and that the amount of the solvent within the fiber is reduced as the fiber is stretched. This would indicate that a more highly drawn fiber would have a higher  $T_g$ ; and it would account for our discovery that a lower temperature is required of the wash for solvent removal where the stretch ratio is lower than where fibers are stretched to a greater extent.

The applicability of the second order transition theory to the practice of the instant invention is largely theoretical inasmuch as it is obviously impractical to measure glass temperatures of transition state fibers during the washing and stretching operation. Whatever the reason, it has been found that substantially all residual solvents can be removed from acrylic fibers, after the spinning

of the solution of acrylic polymer in an organic solvent into a coagulating bath of any type, by simultaneously stretching the coagulated fiber and washing it with water at a temperature not exceeding a given maximum for a given stretch ratio, as follows:

|                  |       | Maximum temperature, °C. |
|------------------|-------|--------------------------|
| Stretch ratio:   |       |                          |
| 1.5              | ----- | 65                       |
| 2.0              | ----- | 75                       |
| 3.0              | ----- | 80                       |
| 4.0 <sup>1</sup> | ----- | 85                       |

<sup>1</sup> Maximum permissible temperature does not increase at stretch ratios above four.

The application of the instant invention to any process, and particularly processes employing the aqueous type coagulation bath, is limited, of course, to the maximum permissible orientation stretch of the particular fiber.

## BRIEF DESCRIPTION OF THE DRAWING

To further understand the invention reference will be made to the attached drawing that forms part of the present application.

In the drawing, the figure is a side elevation view, partly in section, showing schematically an apparatus arrangement of a type which can be used in carrying out the process of the instant invention.

## DESCRIPTION OF THE PREFERRED EMBODIMENT

By "acrylonitrile polymer" is meant polyacrylonitrile, copolymers, including terpolymers and higher interpolymers of acrylonitrile, and blends of polyacrylonitrile and copolymers of acrylonitrile with other polymeric materials, such as polystyrene, polyvinylchloride or other acrylonitrile copolymers. In general, a polymer made from a monomeric mixture of which acrylonitrile is at least 70 percent by weight of the polymerizable content is applicable to the practice of the present invention. Block and graft copolymers of the same general type are within the purview of the invention. Suitable other monomers include vinyl acetate, and other vinyl esters of monocarboxylic acids, vinyl chloride and other vinyl halides, dimethyl fumarate and other dialkyl esters of fumaric acid, dimethyl maleate and other dialkyl esters of maleic acid, methyl acrylate and other alkyl esters of acrylic acid, styrene, and other vinyl-substituted aromatic hydrocarbons, methyl methacrylate and other alkyl esters of methacrylic acid, vinyl-substituted heterocyclic nitrogen ring compounds, such as the vinyl imidazoles, etc., the alkyl-substituted vinylpyridines, vinyl chloroacetate, allyl chloroacetate, methylallyl chloroacetate, allyl glycidyl ether, methylallyl glycidyl ether, allyl glycidyl phthalate, and the corresponding esters of other aliphatic and aromatic dicarboxylic acids, glycidyl acrylate, glycidyl methacrylate, and other mono-olefinic monomers copolymerizable with acrylonitrile.

Many of the more readily available monomers for polymerization with acrylonitrile form copolymers which are not reactive with some dyestuffs and may therefore be impossible or difficult to dye by conventional techniques. Accordingly, these non-dyeable fiber-forming copolymers may be blended with polymers or copolymers which are in themselves more dye-receptive by reason of their physical structure or by reason of the presence of functional groups chemically reactive with the dyestuff, whereby the dyestuff is permanently bonded to the polymer in a manner which lends resistance to removal thereof by the usual laundering and dry cleaning procedures. Suitable blending polymers may be polyvinylpyridine, polymers of alkyl-substituted vinylpyridine, polymers of other vinyl-substituted N-heterocyclic compounds, the copolymers of the various vinyl-substituted N-heterocyclic compounds and other copolymerizable monomers, particularly acrylonitrile.

Of particular utility are the blends formed of polyacrylonitrile or a copolymer of more than 90 percent acrylonitrile and up to 10 percent vinyl acetate, and a copolymer of vinylpyridine or an alkyl-substituted vinylpyridine and acrylonitrile, the said acrylonitrile being present in substantial proportions to provide heat and solvent resistance, and a substantial proportion of the vinylpyridine or derivatives thereof to render the blend receptive to acid dyestuffs. Of particular utility are the blends of copolymers of 90 to 98 percent acrylonitrile and 10 to 2 percent vinyl acetate and sufficient copolymer of 10 to 70 percent acrylonitrile and 90 to 30 percent vinylpyridine to produce a blended composition with a total of 2 to 10 weight percent vinylpyridine.

The polymers just described may be prepared by any conventional polymerization procedure. The spinning dopes may also be prepared using conventional solvents and the spinning carried out in equipment generally used

in the art. Any conventional coagulation means may be used although the advantages of the present invention are most readily apparent and of greatest economic importance when the fibers are wet spun into a non-aqueous liquid coagulating medium.

Referring now to the figure, a water coagulable solution comprising an acrylonitrile polymer dissolved in N, N-dimethylacetamide, N,N-dimethylformamide, dimethylsulfoxide, or the like is passed under pressure from a supply tank (not shown) through a conduit 10 and then through a candle filter 11 wherein undissolved particles and foreign materials in the solution are removed. Ordinarily, gear pumps are used to pump the solution through the filter 11 and to meter same to the spinnerette assembly 12. This assembly includes a spinnerette 13 and is suitably disposed below the upper surface of the coagulating liquid 14 contained in trough or bath 15. Fresh liquid 14 is supplied to trough 15 through pipe 18 and is withdrawn therefrom through pipe 20. Liquid 14 may be an aqueous solution of the same solvent as used in preparation of the spinning dope, or a non-aqueous liquid such as kerosene, butyl alcohol or a polyalkylene glycol containing a desirable quantity of the polymer solvent, typically about 5 to 20% of the total liquid. The coagulated filaments are withdrawn by employment of a positively driven roller 21 or other thread advancing means, the peripheral speed of which preferably is synchronized with the extrusion speed so that the filaments during their travel may be attenuated. After passing around roller 21 and an idler roll 22, the filaments are directed into a second trough 23 containing liquid 24. Liquid 24, in this preferred embodiment, is water at a maximum temperature of less than about 86°. It may be circulated slowly, as a bath or rapidly, as a cascade. Fresh liquid is supplied to trough 23 through pipe 25 and is withdrawn through pipe 26. While it is quite possible to employ only a single bath, or alternatively, three or more, two have been illustrated to show a preferred embodiment including alternative subsequent treatments. The filaments before emerging from the liquid in second trough 23 and being directed around a set of positively driven rolls identified by numerals 27 and 28 are passed under guides 30 and 31. The peripheral speed of rollers 27 and 28 are adjusted so that a predetermined orientation stretch will be imparted to the filaments 16 during their travel in second trough 23.

The washing operation can be accomplished in more than one stage of the process and by employment of other known washing means. However, in this invention the temperature of liquid 24 and the stretch imparted to fiber 16 between rollers 20 and 27, are critical. Minimum travel time and distance of fiber 16 in the critically controlled wash bath, for the accomplishment of the objective of this invention, will vary with the turbulence of the bath, the amount of stretch imparted to the fiber, as well as the number of, and distance between individual filaments. Additional and subsequent washing of the fiber may be at higher or lower temperatures.

To roller 27 additional washing liquid such as hot water may be supplied from a spray or shower head 32, the liquid being collected in a container or tray 33. After leaving rollers 27 and 28, the filaments may be directed through a third trough 34 by being passed under guides 35 and 36. The liquid 37 in this trough is normally water, and, as with the water applied from spray or shower head 32, may or may not conform in temperature to that of bath 24. In addition to further washing of the fibers, bath 37 may serve a variety of purposes. It may be used as a situs to relax and shrink the fiber thereby imparting dimensional stability, in which case the filaments are withdrawn from trough 34 by means of driven roller 38 and associated idler roller 40 operated at a peripheral speed less than that of the peripheral speed of rollers 27 and 28. The bath may be used to impart a further stretch to the fiber resulting in a finer denier filament, in which case the fiber will of course be withdrawn from the bath at a

higher speed than the speed of entry. The bath may also be used to heat set the fiber under constant tension in boiling water in which case the fibers would be withdrawn from the bath at the same speed as the speed of entry. Each of the above additional uses of bath 37 would involve temperatures of the liquid in excess of the maximum critical temperature of liquid 24. Fresh water is supplied to trough 34 through an inlet pipe 41 and is withdrawn through outlet pipe 42. The filaments may then be passed through a finish bath liquid 43 contained in a vessel 44 and composed of a lubricant or like beneficial treating agent. The filaments after being withdrawn from liquid 43 are dried. As illustrated in FIGURE 1 the filaments are continuously directed around a pair of driven drying drums 45 and 46 heated internally with steam or the like. Thereafter the filaments are subjected to additional operations such as crimping and then are collected in the form of continuous filament yarn, tow, or they may be cut to staple fibers.

#### EXAMPLES

Four polymeric compositions are selected as demonstrative of the breadth of the invention: A is a binary copolymer of acrylonitrile, B is a terpolymer, C is a blend of two acrylonitrile copolymers, and D is a blend of the same two copolymers with a polyvinylchloride homopolymer. Spin dopes were prepared from each of these polymeric compositions by dissolving in an appropriate quantity of N,N-dimethylacetamide to provide solutions of satisfactory viscosity for spinning. Compositions and physical properties are given in Table I below.

then spun into filaments under identical conditions except that the temperature of the water in the cascade was maintained at a maximum of 85° C. The results of solvent analysis on the dried filaments are given in Table 3.

TABLE 3

|          | Polymer | Percent solvent in dried fiber |
|----------|---------|--------------------------------|
| Example: |         |                                |
| 5.....   | A       | .23                            |
| 6.....   | B       | .25                            |
| 7.....   | C       | .31                            |
| 8.....   | D       | .30                            |

20 In each of these examples, the residual solvent level has been reduced to about one sixth of the levels shown in Table 2 and is now at a commercially acceptable low level.

25 Further experimentation resulted in the discovery that at lower stretch ratios the maximum permissible temperature of the washing medium is also reduced. During these experiments it was also found that the maximum temperature of the water at any point in the washing cascade was controlling, notwithstanding possible lower temperatures at other points in the cascade. These critical tem-

TABLE I

| Composition                                                                                                 | Polymer Nsp                  | Polymer Tg, °C. | Dope solids, percent |
|-------------------------------------------------------------------------------------------------------------|------------------------------|-----------------|----------------------|
| Polymer:                                                                                                    |                              |                 |                      |
| A..... 94% acrylonitrile, 6% vinyl acetate.....                                                             | 0.165 -----                  | 87              | 24                   |
| B..... 89.8% acrylonitrile, 7.5% vinyl acetate, 2.7% vinyl bromide.....                                     | 0.155 -----                  | 87              | 25                   |
| C..... {93% acrylonitrile, 7% vinyl acetate (88%)<br>50% acrylonitrile, 50% methylvinyl pyridine (12%)..... | 0.267 } 0.255<br>0.155 ----- | 86              | 18                   |
| D..... 87% Blend C, 13% polyvinylchloride.....                                                              | 0.24 -----                   | 86              | 19                   |

As a demonstration of the conventional prior art, the several dopes were then individually spun using conventional equipment into a nonaqueous coagulating bath maintained at 95° C. and consisting essentially of a polyethylene glycol of average molecular weight 1000 and approximately 10% of N,N-dimethylacetamide. The filaments so formed were withdrawn from the coagulating bath after a travel therein of 20" and thereafter directed through a boiling water cascade twenty feet in length and wherein the fibers were stretched to 4.0 times their initial length. The filaments were then dried on rotating drums maintained at a temperature of 125° C. Samples of the dried filaments were analyzed for solvent content, the results of which are shown in Table 2.

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9

TABLE 5

| Example: | Maximum cascade water temp., °C. | Cascade stretch | Percent solvent in dried fiber |
|----------|----------------------------------|-----------------|--------------------------------|
| 13       | 95                               | 2.0             | 1.44                           |
| 14       | 90                               | 2.0             | 1.12                           |
| 15       | 85                               | 2.0             | .97                            |
| 16       | 80                               | 2.0             | 1.00                           |
| 17       | 75                               | 2.0             | .22                            |
| 18       | 95                               | 4.6             | 1.07                           |
| 19       | 85                               | 4.6             | .14                            |
| 20       | 75                               | 4.6             | .16                            |
| 21       | 75                               | 1.5             | .68                            |
| 22       | 75                               | 1.36            | .96                            |
| 23       | 75                               | 2.4             | .13                            |

Any departure from the description herein that conforms to the present invention is intended to be included within the scope of the claims.

We claim:

1. In a process of producing a filament from an acrylonitrile polymer wherein the said polymer is dissolved in a solvent and a stream of the resulting solution is extruded through a spinnerette and thereafter directed into a coagulating bath, and wherein the resulting solvent-laden filament is withdrawn from the coagulating bath and stretched in a water bath to orient the polymer molecules thereof after which the filament is dried and collected, the improvement of maintaining the water bath at just below the glass transition temperature of the filament at the imparted stretch ratio, whereby the filament is rendered substantially solvent-free.

2. The process improvement of claim 1 wherein the filament is stretched at least about 4 times.

3. The process improvement of claim 1 wherein the temperature of the water bath is less than about 81° C. and the filament is stretched at least about 3 times.

4. The process improvement of claim 1 wherein the temperature of the water bath is less than about 76° C. and the filament is stretched at least about 2 times.

5. The process improvement of claim 1 wherein the temperature of the water bath is less than about 66° C. and the filament is stretched at least about 1.5 times.

6. In a process of producing a filament from an acrylonitrile polymer wherein the polymer is dissolved in

5 a solvent, and a stream of the resulting solution is extruded through a spinnerette and thereafter directed into a coagulating bath, and wherein the resulting filament is withdrawn from the coagulating bath, stretched for orientation in the presence of a liquid medium, washed, and dried, the improvement comprising combining the draw step with the wash step by using as a draw bath, a water bath at just below the glass transition temperature of the filament at the imparted stretch ratio, whereby the solvent-laden filament is simultaneously stretched and rendered substantially solvent-free.

10 7. The process improvement of claim 6 wherein the temperature of the water bath is below about 86° C., and the filament is stretched at least about 4×.

8. The process improvement of claim 6 wherein the temperature of the water bath is less than about 81° C. and the filament is stretched at least about 3×.

9. The process improvement of claim 6 wherein the temperature of the water bath is less than about 76° C. and the filament is stretched at least about 2×.

10. The process improvement of claim 6 wherein the temperature of the water bath is less than about 66° C. and the filament is stretched at least about 1.5×.

25

#### References Cited

##### UNITED STATES PATENTS

|           |         |         |           |
|-----------|---------|---------|-----------|
| 2,716,586 | 8/1955  | Terpay  | 264—182   |
| 2,723,900 | 11/1955 | Hooper  | 264—182   |
| 3,088,188 | 5/1963  | Knudsen | 264—182 X |

30

##### FOREIGN PATENTS

|             |         |        |
|-------------|---------|--------|
| 41/20,414   | 11/1966 | Japan. |
| 38/23,264   | 11/1963 | Japan. |
| 35 37/3,920 | 6/1962  | Japan. |
| 39/22,042   | 10/1964 | Japan. |
| 40/1,825    | 2/1965  | Japan. |

JULIUS FROME, Primary Examiner

J. H. WOO, Assistant Examiner

U.S. CL. X.R.

264—182, 203, 210